

Oct. 20, 1931.

J. E. PERRY

1,828,200

INGOT MOLD AND METHOD OF MAKING SAME

Original Filed June 18, 1926



INVENTOR  
*John E. Perry*  
BY  
*George Ramaey*  
his ATTORNEY

## UNITED STATES PATENT OFFICE

JOHN EDMUND PERRY, OF SHARON, PENNSYLVANIA, ASSIGNOR TO VALLEY MOULD AND IRON CORPORATION, OF SHARPSVILLE, PENNSYLVANIA, A CORPORATION OF NEW YORK

## INGOT MOLD AND METHOD OF MAKING SAME

Original application filed June 18, 1926, Serial No. 116,793. Divided and this application filed December 16, 1926. Serial No. 155,133.

The present invention relates to metallurgy and more particularly to ingot molds. This is a division of my pending application, Serial No. 116,793, filed June 18, 1926, which eventuated into Patent 1,643,419, granted September 27, 1927, in which is claimed a set-up and core bar structure. The present invention relates more especially to ingot molds of the closed bottom type. Big-end-up ingot molds adapted for use without stools and being provided in the bottom with a stripping opening usually closed with a plug are known in the art as "closed bottom ingot molds."

Heretofore in the art, it has been customary to cast a closed bottom ingot mold inverted over an inverted sand core; that is, with the bottom of the mold uppermost and with the mouth of the ingot mold being in the bottom of the casting set-up. This results in the impurities rising during casting and leaves the kish and spongy metal in that part of the finished mold which is subjected to greatest strain when the ingot mold is being used to cast steel ingots. Furthermore, this prior method necessitated machining the bottom of the finished ingot mold in order to provide a base surface on which the mold could be set.

The ingot mold comprising the present invention is one wherein the base of the mold is a substantially plane surface adapted to set on a suitable support so that the mold sets with the axis of the matrix substantially vertical. Preferably, the surface on the bottom of the base is a hard skin referred to in the claims as "mold skin", and is produced by contact of the molten metal with the casting mold wall, as distinguished from a surface produced by machining. Machined surfaces add to the cost of the production of the mold and, furthermore, usually cut away the surface skin so that the metal exposed is not as hard as that produced where the hot metal comes into direct contact with the cold wall of the casting mold. More especially, the particular preferred form of the present invention is one wherein this base surface is a chilled surface. This produces hardness conducive to long life of the mold under hard mechanical usage.

The metal in the mold is of the most dense structure adjacent the base of the mold and is of lesser dense structure toward the top of the mold, while the most spongy part of the metal is adjacent the upper end of the mold. This results in a mold having a relatively long metallurgic life in that the bottom portion of the mold, which is subjected to the most severe strains when the mold is heated by molten steel, is good solid metal.

A further attribute of the preferred form of this mold is that the bottom of the matrix thereof shall comprise chilled metal, which is best adapted to receive the direct and full force of the stream of molten steel which initially enters the mold, without being liable to the cut away under the action of this stream of hot metal.

In the method of manufacturing this new mold, in its preferred form, the mold is cast with the bottom downward.

This places the best metal, when cold, in the bottom of the ingot mold and completely obviates machining the base, because the mold seat is automatically formed during the casting operation. The area comprising the bottom of the matrix is chilled either during casting or later. The area comprising the base of the mold is also preferably chilled. The chilling of the bottom of the matrix is of greater importance, however, than the chill on the bottom surface of the base.

It is realized that the present invention may be embodied in constructions other than the specific form herewith disclosed, which is a complete disclosure of the invention as required by the patent statutes. However, realizing that the invention may be utilized and practiced in other forms, it is to be understood that the disclosure herewith is illustrative and not to be considered in the limiting sense.

The figure of the drawing is a vertical sectional view through a mold made in accordance with the present method and invention.

Referring now more specifically to the drawing which illustrates a section through the preferred form of mold comprising chilled dense metal as at 27, and the bottom of the matrix likewise comprises a chill dense

metal as at 28. The most compact, solid and firm metal in the mold is in the bottom portion or zone arbitrarily indicated on the figure in the drawing by means of the lower bracket 29. The next best metal is in the zone arbitrarily indicated by the middle bracket 30; and the metal containing the greatest amount of impurities is in the zone arbitrarily indicated by the upper bracket 31. It is to be understood, of course, that there is no distinct line of demarcation between the zones indicated by the brackets 29, 30 and 31, but that these arbitrary divisions are merely conveniences of expression to set forth the conditions of the metal in the mold having a structure in accordance with the present invention.

The method of manufacturing the preferred form of the present mold comprises casting the mold with the bottom matrix 28 downward so that the initial molten metal poured into the casting set-up forms the bottom portion of the ingot mold. Then, as the molten metal rises to form the sides of the mold, the impurities in the molten metal will rise with the molten metal and certain proportions of these impurities will be trapped in the side walls of the mold as the molten metal freezes. However, the greater the amount of molten metal used in the casting, the greater the percentage of impurities which are floated upwardly through the molten metal and consequently, the upper part of the finished mold will contain the greatest amount of impurities. In the manufacture of the mold in the preferred form, the bottom portion of the matrix preferably is chilled. This chill may be brought about by the introduction of chilling means either during the casting operation or so shortly thereafter as to chill the metal surface at the bottom of the matrix as at 28. Preferably, the base surface of the mold is cast against a forming surface to form a seat for said mold, and preferably, though not necessarily, is chilled by any commonly known method in the art, either during casting or so shortly thereafter that the rapid cooling of the metal will result in chilled metal adjacent this surface when the mold has cooled.

A closed bottom mold in accordance with the present invention has chilled surfaces where the mold is subjected to greatest wear and since these chilled surfaces are adjacent the heaviest mold wall, the strains set up in the ingot mold by the chilling operation are supported by sufficient metal to prevent any tendency of the chilled portions to break down during the use of the mold because of the varying heat conditions to which the mold is subjected while being used to cast steel ingots.

Having thus described my invention, what I claim is:

1. An article of manufacture comprising a cast iron ingot mold having a closed bottom and with the most dense cast iron in the lower portion of the mold adjacent the bottom of the matrix face wall, and with the density of the cast iron decreasing upwardly in such manner that the least dense iron is adjacent the mouth of the mold. 70

2. An article of manufacture comprising a cast iron ingot mold having a closed bottom and with the most dense cast iron in the lower portion of the mold adjacent the bottom of the matrix, the metal adjacent the bottom of the matrix face wall being chilled, and with the density of the cast iron decreasing upwardly in such manner that the least dense iron is adjacent the mouth of the mold. 75

3. An article of manufacture, a cast iron ingot mold having a closed bottom and with the metal comprising the bottom of the matrix being chilled cast iron. 80

4. As an article of manufacture, a closed bottom ingot mold having a smooth chilled base portion, and a smooth chilled surface comprising the face of the bottom of the matrix portion of the mold. 85

5. As an article of manufacture, a cast iron closed bottom ingot mold having a smooth chilled base portion, and a smooth chilled surface comprising the bottom of the matrix portion of the mold, and with the metal of least solidity and density being adjacent the mouth of the mold. 95

6. As an article of manufacture, an ingot mold comprising a cast iron body having a substantially closed bottom matrix, the bottom portion of said matrix comprising chilled metal having a close fine grain, and the base of said mold comprising a smooth portion of chilled mold skin metal. 100

7. As an article of manufacture, an ingot mold comprising a cast iron body having a substantially closed bottom matrix, the bottom portion of said matrix comprising chilled metal having a close fine grain, and the base of said mold comprising a smooth portion of chilled mold skin metal, the most dense metal being in the bottom portion of said mold. 105

8. The method of manufacturing a cast iron closed bottom ingot mold comprising casting the mold with the bottom downward and chilling the cast iron adjacent the bottom of the matrix of the ingot mold. 110

9. The method of manufacturing a cast iron ingot mold having a closed bottom which method comprises chilling the metal adjacent the bottom walls of the matrix and also chilling the metal adjacent the surface comprising the base of the mold. 120

10. A method of manufacturing a cast iron closed bottom ingot mold comprising chilling the metal of the walls adjacent the bottom of the matrix. 125

11. The method of manufacturing a cast iron closed bottom mold having a stripping opening in the bottom of the mold, comprising casting the mold with the closed bottom downwardly and chilling the bottom of the matrix walls and also chilling the metal surrounding the stripping opening.

JOHN EDMUND PERRY.

10

15

20

25

30

35

40

45

50

55

60